# EUROPEAN PATENT SPECIFICATION

(11) **EP 4 323 570 B1**
(45) Date of publication and mention of the grant of the patent: **23.07.2025**
(21) Application number: 22710903.0
(22) Date of filing: 01.03.2022
(51) Int. Cl.: D02G 3/44, D02G 3/32, D02G 3/28, D04B 1/12, D04B 1/28

(54) **FABRIC AND ARTICLES HAVING FIRE-RESISTANCE, CUT-RESISTANCE, AND ELASTIC RECOVERY AND PROCESSES FOR MAKING SAME**
GEWEBE UND ARTIKEL MIT FEUERBESTÄNDIGKEIT, SCHNITTFESTIGKEIT UND ELASTISCHER ERHOLUNG SOWIE HERSTELLUNGSVERFAHREN DAFÜR
TISSU ET ARTICLES PRÉSENTANT UNE RÉSISTANCE AU FEU, UNE RÉSISTANCE AUX COUPURES ET UNE RÉCUPÉRATION ÉLASTIQUE ET LEURS PROCÉDÉS DE FABRICATION

(30) Priority: 12.04.2021 US 202163173697 P
(43) Date of publication of application: 21.02.2024
(73) Proprietor: DuPont Safety & Construction, Inc., Wilmington, DE 19805 (US)
(72) Inventor: HANKS, Jeffrey Alan, Midlothian, Virginia 23112 (US); KEY, Eric, Richmond, Virginia 23224 (US); NOTH, Olivier Beat, 1680 Romont, Fribourg (CH)
(74) Representative: Abitz & Partner
(86) International application number: PCT/US2022/018309
(87) International publication number: WO 2022/220937

(56) References cited:
- US-A- 5 448 779
- US-A1- 2009 183 296
- US-A1- 2015 322 598
- US-B2- 6 952 915

## Description

### Background of the Invention

1. Field of the Invention. This invention relates to yarns and fabrics suitable for use in articles of protective clothing that have fire-resistant and form-fitting properties and also have cut resistant properties.

Description of Related Art. Ply-twisted yarns and fabric having cut-resistance and elastic recovery, processes for making same, and their used in articles of protective clothing is disclosed in United States Pat. No. 6,952,915.

Yarns comprising modacrylic fiber, p-aramid fiber, and m-aramid fiber that are useful for the production of fabrics which possess arc and flame protective properties are disclosed, for example, in United States Pat. Nos. 7,065,950 and 7,348,059. These yarns may further comprise, as an optional component, 2 to 15 weight percent of an abrasion-resistant fiber such as a nylon and/or 1 to 5 weight percent of an antistatic component.

Yarns and fabrics having a combination of fire resistance and elastic recovery properties are described, for example, in United States Pat. Nos. 5,069,957; 5,527,597; and 5,694,981. These existing solutions utilize yarns made by covering elastic core yarns with a substantial protective fiber outer covering made from a fire-resistant fiber. In other words, these references describe protecting the elastic core by structurally shielding the elastic core from flame by use of another fiber that is in the same yarn.

As used herein, the terms "structural shielding" and "structural shield" mean the cover fibers simply char and remain in place in a yarn covering any elastic filaments in the core when exposed to a flame and therefore provide a structural barrier between a flame and the elastic core. As taught in these patents, these yarns are provided with a substantial protective fiber outer covering made from a fire-resistant fiber that physically protects the elastic core yarns from degradation or melting, when exposed to extreme temperatures and fire.

Unfortunately, in many instances, the fibers that provide an adequate structural shielding outer fiber covering also tend to be stiffer fibers, and therefore fabrics made with such yarns can be less comfortable than desired. This ultimately translates to protective apparel that can be less comfortable than desired, and it is well known that workers tend to not wear their protective gear if it is not adequately comfortable, putting themselves at risk.

Additionally, any solution for protecting the elastic core should meet current protective apparel standards. Specifically, the recent NFPA 2112-2018 "Standard on Flame-Resistant Clothing for Protection of Industrial Personnel Against Short-Duration Thermal Exposures from Fire" provides specifications for the minimum design, performance, testing, and certification requirements and test methods for flame-resistant garments, shrouds, hoods, balaclavas, and gloves for use in areas at risk from short-duration thermal exposure from fire. The Standard requires the fabric used in the garments have an afterflame time of not more than 2 seconds. The afterflame time is the time, in seconds, to the nearest 0.2 second, that the specimen continues to flame after the burner is removed from the flame.

The Standard has even more stringent requirements for flame-resistant gloves, in that the material consumed in the flame resistance testing should not exceed 5.0 percent of the specimen's original weight. In other words, after the specified 12 seconds of flame is applied to a specimen per the procedure in the Standard, the fabric weight loss should be 5.0 percent or less.

Therefore, what is needed is a yarn and/or fabric having a combination of fire resistance and elastic recovery properties, along with cut resistance, that specifically incorporates elastic core yarns, that meets the NFPA 2112-2018 Standard; and that further utilizes fibers that have a textile feel to potentially provide a more comfortable protective apparel article.

In the present description the following conversions apply: 1 grams force = 9.8 mN; 1 inch = 25.4 mm; 1 oz/yd² = 33.9 g/m²; 5900/cotton count = dtex; 1 denier = 1.1 dtex.

### Brief Summary of the Invention

This invention relates to a flame-resistant cut-resistant fabric, and a glove or other article comprising the fabric, the fabric comprising:
(a) at least one first yarn comprising at least 50 weight percent heat-resistant polymeric fiber, based on the total weight of the first yarn, wherein at least 30 weight percent of the polymeric fiber present in the at least one first yarn is cut-resistant heat-resistant polymeric fiber having a cut resistance of 500 grams force or higher per ASTM F2992-15; and
(b) at least one second yarn having a sheath/core construction with a sheath of halogenated self-extinguishing staple fibers and a core comprising at least one continuous elastomeric filament,

wherein 60 to 95 weight percent of the at least one second yarn is halogenated self-extinguishing fiber, based on the total weight of the second yarn, and the halogenated self-extinguishing fiber is in contact with the at least one continuous elastomeric filament, the second yarn being free or substantially free of inorganic fibers;
wherein the fabric has a maximum after-flame time of two seconds or less and weight loss of 5 weight percent of less when tested per NFPA-2112-2018.

### Detailed Description of the Invention

This invention relates to yarns and fabrics, suitable for use in articles of protective clothing, that have both fire-resistant and form-fitting properties, and additionally provide cut protection. The unique combination is created by combining elastic materials, self-extinguishing fibers, and strong heat-resistant polymeric fibers in a manner to provide high fire resistance in a yarn or fabric along with limited consumption of the fabric during burning.

Specifically, this invention relates to a flame-resistant cut-resistant fabric, comprising:
(a) at least one first yarn comprising at least 50 weight percent heat-resistant polymeric fiber, based on the total weight of the first yarn, wherein at least 30 weight percent of the polymeric fiber present in the at least one first yarn is cut-resistant heat-resistant polymeric fiber having a cut resistance of 500 grams force or higher per ASTM F2992-15; and
(b) at least one second yarn having a sheath/core construction with a sheath of halogenated self-extinguishing staple fibers and a core comprising at least one continuous elastomeric filament,

wherein 60 to 95 weight percent of the at least one second yarn is halogenated self-extinguishing fiber, based on the total weight of the second yarn, and the halogenated self-extinguishing fiber is in contact with the at least one continuous elastomeric filament, the second yarn being free or substantially free of inorganic fibers;
wherein the fabric has a maximum after-flame time of two seconds or less and weight loss of 5 weight percent of less when tested per NFPA-2112-2018.

By "flame-resistant cut-resistant fabric", it is meant a knitted or woven fabric that is both "flame resistant" and "cut resistant". By the descriptor "flame resistant", in regard to a fabric, it is meant the fabric has a char length equal to or less than 4 inches (100 mm) when tested per ASTM 6143-15. By "cut resistant fabric", it is meant the fabric has at least a minimum level of cut resistance, and generally a cut-resistant fabric has a cut resistance of at least 200 grams force per ASTM F2992-15. According to the invention, the fiber and yarns described herein can provide a flame-resistant cut-resistant fabric having a cut resistance of at least 500 grams force per ASTM F2992-15. However, it is understood that in some other embodiments, other fibers or yarns that don't necessarily provide cut resistance but may provide other desirable qualities to the fabric may be incorporated into the fabric as long as the flame performance requirements describe herein to be considered a "flame-resistant" fabric are met and the fabric retains a minimum cut-resistance of at least 200 grams force per ASTM F2992-15.

Flame-resistant fabrics provide thermal protection from thermal events, while cut resistant fabrics provide mechanical protection from such things as knives and sharp edges. The fabric, in addition to being flame resistant, has an afterflame time of two seconds or less and weight loss of 5 weight percent of less when tested per NFPA-2112-2018.

In addition, it is often important or desirable for any articles, such as protective gloves, that are made from such fabrics be comfortable and have good fit and dexterity. By "good fit and dexterity" it is meant, for example, that gloves conform nicely to the shape of the hands of the wearer and one is able to pick up and manipulate small objects while wearing the gloves. The flame-resistant cut-resistant fabrics as described herein are both highly flame-resistant and cut-resistant, while also providing articles that are soft, flexible, and form fitting. Protective apparel made from such fabrics is very comfortable and effective against multiple threats.

The flame-resistant cut-resistant fabric is made from at least a first yarn that provides a heat-resistant polymeric fiber and at least a second yarn that provides at least one continuous elastomeric filament covered by halogenated self-extinguishing fiber that is in contact with the at least one continuous elastomeric filament. The at least first yarn and the at least second yarn are then used to make the fabric.

In some embodiments, the at least first yarn and the at least second yarn are twisted together to form a ply-twisted yarn. In some embodiments, the ply-twisted yarn consists of only one first yarn and only one second yarn. In other embodiments, the ply-twisted yarn consists of only one first yarn and a plurality of second yarns; and in other embodiments, the ply-twisted yarn consists of a plurality of first yarns and only one second yarn. Likewise, in some embodiments the ply-twisted yarn consists of a plurality of first yarns and a plurality of second yarns. Finally, in some embodiments, the ply-twisted yarn comprises at least one first yarn and at least one second yarn; other yarns made from any number of fibers can be included in ply-twisted yarn as long the final fabric meets the performance criteria discussed herein.

In some other embodiments the at least first yarn and the at least second yarn are used in a co-knitted weft insertion structure. By "weft insertion" it is meant a knit wherein the at least second yarn is inserted into a knitted structure comprising the at least first yarn, such as is done in making elastomeric cuffs in knit gloves.

In some other embodiments the at least first yarn and the at least second yarn or can be used in a parallel relationship to each other in the fabric. The word "parallel", as used herein, means that the individual yarns are generally present in the fabric next to each other side-by-side and that the yarns are independent and separate from each other, they are not plied or twisted together. In knit fabrics, this type of parallel arrangement in the fabric is also known as one type of co-knit fabric. In one co-knit manufacturing process, the co-knit is formed by knitting the two separate yarns two-ends-in, i.e., both together, on a single knitting machine. This structure and process maintains the two different yarns in close proximity in the fabric, maintaining their parallel relationship. The process can advantageously include the step of plaiting the two ends of yarn during knitting to locate one of the ends predominantly at a first surface of a garment, and the other of the ends predominantly at a second surface of the garment. This allows placing of the typically more comfortable end predominantly on the inside of a garment and locating the other predominantly on the outside.

This invention also relates to a glove or other article comprising a flame-resistant cut-resistant fabric including all of the embodiments described herein, the flame-resistant cut-resistant fabric comprising:
(a) at least one first yarn comprising at least 50 weight percent heat-resistant polymeric fiber, based on the total weight of the first yarn, wherein at least 30 weight percent of the polymeric fiber present in the at least one first yarn is cut-resistant heat-resistant polymeric fiber having a cut resistance of 500 grams force or higher per ASTM F2992-15; and
(b) at least one second yarn having a sheath/core construction with a sheath of halogenated self-extinguishing staple fibers and a core comprising at least one continuous elastomeric filament,

wherein 60 to 95 weight percent of the at least one second yarn is halogenated self-extinguishing fiber, based on the total weight of the second yarn, and the halogenated self-extinguishing fiber is in contact with the at least one continuous elastomeric filament, the second yarn being free or substantially free of inorganic fibers;
wherein the fabric has a maximum after-flame time of two seconds or less and weight loss of 5 weight percent of less when tested per NFPA-2112-2018.

The at least one first yarn comprises at least 50 weight percent heat-resistant polymeric fiber, based on the total weight of the first yarn, wherein at least 30 weight percent of the polymeric fiber present in the at least one first yarn is cut-resistant heat-resistant polymeric fiber having a cut resistance of 500 grams force or higher per ASTM F2992-15.

By "heat resistant polymeric fiber", it is meant a fiber made from a synthetic organic polymer that retains 90 percent of its original fiber weight when heated in air to 500° C at a rate of 20° C. per minute. Preferred heat resistant polymeric fibers have a yarn tenacity of at least 3 grams per denier (2.7 grams per dtex). Heat resistant polymeric fibers include para-aramid fibers, aramid copolymer fibers, polybenzazole fibers, polybenzimidazole fibers, polyimide fibers, and mixtures thereof. Preferred heat resistant polymeric fibers are para-aramid fibers, and the preferred para-aramid fiber is poly(paraphenylene terephthalamide fiber.

The at least one first yarn comprises at least 50 weight percent heat-resistant polymeric fiber based on the total weight of the first yarn. In some embodiments, the at least one first yarn comprises at least 60 weight percent heat-resistant polymeric fiber based on the total weight of the first yarn. In some embodiments, the at least one first yarn comprises 60 to 85 weight percent heat-resistant polymeric fiber based on the total weight of the first yarn, and in some other embodiments, the at least one first yarn comprises 60 to 80 weight percent heat-resistant polymeric fiber, based on the total weight of the first yarn. In some embodiments, the at least one first yarn comprises 100 weight percent heat-resistant polymeric fiber based on the total weight of the first yarn.

At least 30 weight percent of the polymeric fiber present in the at least one first yarn is cut-resistant heat-resistant polymeric fiber having a cut resistance of 500 grams force or higher per ASTM F2992-15. The cut performance of a fiber is determined by measuring the cut performance of a 345 grams/square meter (10 ounces/square yard) fabric that is woven or knitted from 100% of the fiber to be tested, and then the cut resistance (in grams-force) is measured by-ASTM F2992-15.

Cut-resistant heat-resistant polymeric fiber having a cut resistance of 500 grams-force or higher per ASTM F2992-15 include para-aramid fibers, aramid copolymer fibers, polybenzazole fibers, polybenzimidazole fibers and mixtures thereof. Preferred cut-resistant heat-resistant polymeric fibers are para-aramid fibers, and the preferred para-aramid fiber is poly(paraphenylene terephthalamide fiber. The cut-resistant heat-resistant polymeric fiber in the at least one first yarn can be the same or different from the heat-resistant polymeric fiber in the at least one first yarn, if the heat-resistant polymeric fiber has adequate cut-resistance.

Therefore, it is understood that cut-resistant heat-resistant polymeric fiber is both a heat-resistant polymeric fiber as previously defined and a cut-resistant fiber as previously defined. Further, the at least one first yarn can be 100% cut-resistant heat-resistant polymeric fiber. That is, it is understood that such a yarn having 100% cut-resistant heat-resistant polymeric fiber has therefore at least 50 weight percent heat-resistant polymeric fiber and also at least 30 weight percent cut-resistant heat resistant polymeric fiber. It is also understood that the at least one first yarn can include fiber that is heat-resistant polymeric fiber as defined herein but is not cut-resistant fiber as defined herein. Table 1 provides a guide, giving selected example compositions, as to the possible percentages of non-cut-resistant heat-resistant (Non-CR HR) polymeric fiber and cut-resistant heat-resistant (CH-HR) polymeric fiber.

**Table 1**

| **Total HR Fiber in First Yarn (wt%)** | **Minimum Amount of Non-CR HR Fiber (wt%)** | **Maximum Amount of CR-HR fiber (wt%)** | **Maximum Amount of Non-CR HR fiber (wt%)** | **Minimum amount of CR-HR fiber (wt%)** | **Total Non-HR Fiber in First Yarn (wt%)** |
|---|---|---|---|---|---|
| 50 | 0 | 50 | 20 | 30 | 50 |
| 60 | 0 | 60 | 30 | 30 | 40 |
| 70 | 0 | 70 | 40 | 30 | 30 |
| 80 | 0 | 80 | 50 | 30 | 20 |
| 90 | 0 | 90 | 60 | 30 | 10 |
| 100 | 0 | 100 | 70 | 30 | 0 |

Therefore, it is understood that the at least 30 weight percent of the polymeric fiber present in the at least one first yarn is both a cut-resistant and heat-resistant polymeric fiber as defined herein. In some embodiments, the cut-resistant heat-resistant polymeric fiber is present in the at least one first yarn in an amount of 50 weight percent to 100 weight percent, based on the total amount of polymeric fiber in the at least one first yarn. In some other embodiments, the cut-resistant heat-resistant polymeric fiber is present in the at least one first yarn in an amount of 80 weight percent to 100 weight percent, based on the total amount of polymeric fiber in the at least one first yarn. In other embodiments, the cut-resistant heat-resistant polymeric fiber is present in the at least one first yarn in an amount of 80 weight percent to 95 weight percent, based on the total amount of polymeric fiber in the at least one first yarn

In addition to the various example percentages of cut-resistant heat-resistant polymeric fiber and non-cut resistant heat-resistant polymeric fiber shown in Table 1, in some embodiments, the at least one first yarn further comprises other synthetic or organic fibers or filaments that are not heat-resistant polymeric fiber; that is, they do not meet the definition of a heat-resistant polymeric fiber provided herein. Essentially any type of fiber can be included as long as long the final fabric meets the compositions described herein and the performance criteria discussed herein. That is, the composition of the at least one first yarn comprises at least 50 weight percent heat-resistant polymeric fiber, based on the total weight of the polymeric fiber in the first yarn, and wherein at least 30 weight percent of the polymeric fiber is cut-resistant heat-resistant fiber; and the final fabric is a flame resistant fabric as defined herein and has a maximum after-flame time of two seconds or less and weight loss of 5 weight percent of less when tested per NFPA-2112-2018. Preferably, the fibers or filaments that are not heat-resistant polymeric fiber are organic fibers and in some embodiments are polymeric organic fibers. Also, in some embodiments, if present, the fibers or filaments that are not heat-resistant polymeric fiber are synthetic or organic staple fibers.

In some preferred embodiments, the at least one first yarn can further comprise flame-resistant fiber. By "flame-resistant fiber", it is meant that a fabric made solely from that fabric has a char length equal to or less than 4 inches and an afterflame equal to or less than 2 seconds per the vertical flame test of ASTM D6143-99; but the fabric does not meet the cut-resistance criteria previously described herein for cut-resistant heat-resistant polymeric fibers. Suitable flame-resistant fibers include meta-aramid fibers, with the preferred meta-aramid being poly(metaphenylene isophthalamide). Other potentially useful flame-resistant fiber could include blends of meta-aramids and flame-retardant-treated (FR) cellulose, FR cotton, FR lyocell, or mixtures thereof. In some embodiments, the at least one first yarn has 30 to 70 weight percent flame-resistant fiber, based on the total weight of the polymeric fiber in the first yarn. In some other preferred embodiments the at least one first yarn has 50 to 70 weight percent flame-resistant fiber, based on the total weight of the polymeric fiber in the first yarn.

Both the heat-resistant polymeric fiber and the cut-resistant heat-resistant polymeric fiber in the at least one first yarn are staple fibers preferably having a length of about 2 to 20 centimeters, preferably about 3.5 to 6 centimeters. Both the heat-resistant polymeric fiber and the cut-resistant heat-resistant polymeric fiber in the at least one first yarn are staple fibers preferably having a diameter of 5 to 25 micrometers and a linear density of 0.5 to 7 dtex. Also, in some embodiments, if present, the fibers or filaments that are flame resistant fibers or are not heat-resistant polymeric fiber are staple fibers having dimensions similar to the above ranges for the heat-resistant polymeric fiber and the cut-resistant heat-resistant polymeric fiber.

In some embodiments, the at least one first yarn comprising at least 50 weight percent heat-resistant polymeric fiber, based on the total weight of the first yarn, and wherein at least 30 weight percent of the polymeric fiber present in the at least one first yarn is cut-resistant heat-resistant polymeric fiber having a cut resistance of 500 grams force or higher per ASTM F2992-15, the at least one first yarn further having a sheath/core construction with the sheath comprising the cut-resistant heat-resistant polymeric fiber and the core comprising an inorganic fiber. When an application desires or requires superior cut resistance, at least one inorganic fiber is preferably added to the yarn. The sheath/core construction is used because the sheath staple fibers provide a cover and shield the inorganic filament in the core from direct abrasive contact with the skin giving the fabrics containing the sheath/core yarn improved comfort.

In some embodiments when the inorganic fiber is present in the at least one first yarn, the inorganic fiber is present in an amount of 15 to 40 weight percent of the total weight of the first yarn. Likewise, the maximum amount of the heat-resistant polymeric fiber in these sheath-core first yarns when the inorganic fiber is present is 85 weight percent, based on the total weight of the first yarn. In some preferred embodiments, the sheath/core yarns have 60 to 80 weight percent heat-resistant polymeric fiber in the sheath and 20-40 weight percent organic fiber in the core. Preferably the inorganic fiber in the core is a steel or tungsten. Preferably, the fiber in the core is present as one or more continuous filaments.

The sheath fiber can be wrapped or spun around the inorganic filament core. Specifically, this can be achieved by known means, such as, conventional ring spinning including improvements to the conventional process such as those utilizing COTSON technology; core-spun spinning such as DREF spinning; air-jet spinning using so-called core insertion with Murata (now Muratec) jet-like spinning; open-end spinning, and the like. Preferably the staple fiber is consolidated around the inorganic filament core at a density sufficient to cover the core. The degree of coverage depends on the process used to spin the yarn; for example, core-spun spinning such as DREF spinning (disclosed, for example, in U.S. Pat. Nos. 4,107,909; 4,249,368; & 4,327,545) provides better coverage than ring spinning. Conventional ring spinning provides only partial coverage of the center core, but even partial coverage can provide adequate sheath/core coverage. The sheath can also include some fibers of other materials to the extent that decreased cut resistance, due to that other material, can be tolerated

The incorporation of the at least one inorganic filament as the core in this embodiment of the first yarn can be achieved, for example in its simplest practical application, by passing a roving, sliver, or collection of the heat-resistant and cut resistant fibers, and optionally the non-heat resistant fibers through sets of drafting rolls to make a drafted fiber mass to be ring twisted into a single yarn. The at least one inorganic filament is typically fed from a bobbin through a set of feed rolls and subsequently into the staple fibers prior to the final set of drafting rollers. Since the inorganic core filament(s) are not elastomeric they do not have to be over-tensioned during insertion into the yarn, with only enough tension applied to either the sheath fibers and the core as is conventionally used.

The at least one first yarn in the form of a sheath/core yarn generally comprises 15-50 weight percent inorganic filament(s) with a total linear sheath/core yarn density of 100 to 5000 dtex. The core comprising an inorganic fiber can be a single filament, or may be multifilament, and is preferably a single metal filament or several metal filaments, as needed or desired for a particular application or degree of cut protection. By metal filament is meant filament or wire made from a ductile metal such as stainless steel, copper, aluminum, bronze, tungsten and the like, or metal fiber constructions commonly known as "micro-steel". Stainless steel is the preferred metal. The metal filaments are generally continuous wires. Useful metal filaments are 1 to 150 micrometers in diameter and are preferably 25 to 75 micrometers in diameter.

In some embodiments, the inorganic fiber is a glass filament. It can be one or more glass filaments, such as for example 110 dtex(100 denier) glass filament. However, glass is less preferred because it has less cut resistance per linear density than metal and it is much more critical that the glass be substantially covered by the staple fiber sheath to minimize skin irritation should the yarn be used in gloves, sleeves, etc., where the fabric is in contact with the skin. Therefore, in many embodiments the inorganic fiber is a metal filament.

Again, it is understood that for these sheath/core yarns, the cut-resistant heat-resistant polymeric fiber is both a heat-resistant polymeric fiber as previously defined and a cut-resistant fiber as previously defined. It is also understood that the at least one first yarn can include fiber that is heat-resistant polymeric fiber as defined herein but is not cut-resistant fiber as defined herein. Table 2 provides a guide, giving selected example compositions, as to the possible percentages of total heat-resistant (CH-HR) polymeric fiber and total inorganic filament in the at least one first yarn, and further provides possible percentages illustrating possible amounts of non-cut-resistant heat-resistant (Non-CR HR) polymeric fiber and cut-resistant heat-resistant (CH-HR) polymeric fiber.

**Table 2**

| **Total HR Fiber (all types) in First Yarn (wt%)** | **Minimum Amount of Non-CR HR Fiber (wt%)** | **Maximum Amount of CR-HR Fiber (wt%)** | **Maximum Amount of Non-CR HR Fiber (wt%)** | **Minimum Amount of CR-HR Fiber (wt%)** | **Total Inorganic Filament in First Yarn (wt%)** |
|---|---|---|---|---|---|
| 50 | 0 | 50 | 20 | 30 | 50 |
| 60 | 0 | 60 | 30 | 30 | 40 |
| 70 | 0 | 70 | 40 | 30 | 30 |
| 80 | 0 | 80 | 50 | 30 | 20 |
| 85 | 0 | 85 | 55 | 30 | 15 |

The at least one second yarn has a sheath/core construction with a sheath of halogenated self-extinguishing staple fibers and a core comprising at least one continuous elastomeric filament, wherein 60 to 95 weight percent of the at least one second yarn is halogenated self-extinguishing fiber, based on the total weight of the second yarn, and the halogenated self-extinguishing fiber is in contact with the at least one continuous elastomeric filament, the second yarn being free or substantially free of inorganic fibers.

The at least one second yarn has a sheath/core construction, with the sheath of halogenated self-extinguishing staple fibers being in contact with and covering the core of the at least one continuous elastomeric filament. It is believed that the halogenated self-extinguishing staple fibers provide an active flame-extinguishing cover for the core of the at least one continuous elastomeric filament. This is unlike cover fibers that provide "structural shielding" of the core, that is, cover fibers that simply char and remain in place when exposed to a flame and therefore provide a structural barrier between a flame and the elastic core. Instead, the sheath of halogenated self-extinguishing staple fibers decomposes in the presence of high thermal flux as in a flame, releasing a halogen gas that displaces localized oxygen from the yarn and hinders the burning of the core of the at least one continuous elastomeric filament. Therefore, it is believed that halogenated self-extinguishing staple fibers should not only cover the core but be in direct contact with the core to locally displace oxygen from the surface of the core of the at least one continuous elastomeric filament.

The sheath of halogenated self-extinguishing staple fibers can be wrapped or spun around the at least one continuous elastomeric filament. This can be achieved by known means, such as, conventional ring spinning including improvements to the conventional process such as those utilizing COTSON technology; core-spun spinning such as DREF spinning; air-jet spinning using so-called core insertion with Murata (now Muratec) jet-like spinning; open-end spinning, and the like. Preferably the staple fiber is consolidated around the core of at least one continuous elastomeric filament at a density sufficient to cover the core. The degree of coverage depends on the process used to spin the yarn; for example, core-spun spinning such as DREF spinning (disclosed, for example, in U.S. Pat. Nos. 4,107,909; 4,249,368; & 4,327,545) provides better coverage than ring spinning. Conventional ring spinning provides only partial coverage of the center core, but even partial coverage is assumed a possible sheath/core structure herein.

It is believed the flame-extinguishing effect of the halogenated self-extinguishing staple fibers is adequate when 60 to 95 weight percent of the at least one second yarn is halogenated self-extinguishing fiber, based on the total weight of the second yarn. In some embodiments, it is desirable for 80 to 95 weight percent of the at least one second yarn to be the halogenated self-extinguishing fiber, based on the total weight of the second yarn. The sheath can also include some fibers of other materials to the extent that decreased flame-extinguishing effect, due to that other material, can be tolerated
Halogenated self-extinguishing fibers include those made from halogenated polymer. One especially preferred halogenated self-extinguishing fiber is a fiber made from a modacrylic polymer. By "modacrylic polymer" it is meant preferably the polymer is a copolymer comprising 30 to 70 weight percent of acrylonitrile and 70 to 30 weight percent of a halogen-containing vinyl monomer. The halogen-containing vinyl monomer is at least one monomer selected, for example, from vinyl chloride, vinylidene chloride, vinyl bromide, vinylidene bromide, etc.

In some embodiments the modacrylic copolymers are those of acrylonitrile combined with vinylidene chloride. In some embodiments, the modacrylic copolymer has in addition antimony oxide or antimony oxides. In some preferred embodiments the modacrylic copolymer has either less than 1.5 weight percent antimony oxide or antimony oxides, or the copolymer is totally free of antimony. Very low antimony content polymer and antimony-free polymer can be made by restricting the amount of, or eliminating entirely, any antimony compounds added to the copolymer during manufacture. Representative processes for modacrylic polymers, including those that can be modified in this manner are disclosed in U.S. Pat. No. 3,193,602 having 2 weight percent antimony trioxide; U.S. Pat. No. 3,748,302 made with various antimony oxides that are present in an amount of at least 2 weight percent and preferably not greater than 8 weight percent; and U.S. Pat. Nos. 5,208,105 & 5,506,042 having 8 to 40 weight percent of an antimony compound. In some embodiments, the modacrylic polymer has an LOI of at least 26. In one preferred embodiment the modacrylic polymer has a LOI of at least 26 while also being antimony-free.

The halogenated self-extinguishing staple fibers in the at least one second yarn are staple fibers preferably having a length of about 2 to 9 centimeters, preferably about 3.5 to 6 centimeters. The halogenated self-extinguishing staple fibers in the at least one second yarn are staple fibers preferably having a diameter of 5 to 25 micrometers and a linear density of 0.5 to 7 dtex.

The fabric contains at least one second yarn having a sheath/core construction with a sheath of halogenated self-extinguishing staple fibers and a core comprising at least one continuous elastomeric filament. The halogenated self-extinguishing fiber is in contact with the at least one continuous elastomeric filament, eliminating the need for the entire surface of the elastomeric filament(s) to actually be fully covered by the staple fiber sheath.

In some embodiments, preferably at least 90% of the core is covered by the sheath, as viewed under a microscope with the yarn in a relaxed condition; that is, wherein the sheath-core yarn is viewed when not under tension. The actual covering of the core can depend on the degree the yarn is tensioned; however, it is believed the modacrylic provides its shielding benefit as long as it is in contact with the elastomeric core.

In some embodiments, 5 to 40 weight percent of the total weight of the at least one second yarn is the at least one continuous elastomeric filament. In some embodiments, a ring-spun second yarn has a core comprising at least one elastomeric filament and a partially covering of halogenated self-extinguishing staple fibers. In some preferred embodiments, the core of elastomeric filament(s) comprises 5 to 25 weight percent of the total sheath/core single yarn linear density of 100 to 1500 dtex.

A "core comprising at least one continuous elastomeric filament", as used herein, means a core formed from or containing filaments of an elastomer, the core preferably having the ability to return to its original length rapidly after repeated stretching, even to at least twice its original length. Preferred elastomeric cores include polyurethane based yarns such as spandex or elastane; however, any fiber generally having stretch and recovery can be used. Suitable well-known elastomeric yarns also include the products sold under the tradenames Dorlastan^{®} and Lycra^{®}.

The preferred at least one continuous elastomeric filament is spandex fiber. As used herein, "spandex" has its usual definition, that is, a manufactured fiber in which the fiber-forming substance is a long chain synthetic polymer composed of at least 85% by weight of a segmented polyurethane. Among the segmented polyurethanes of the spandex type are those described in, for example, U.S. Pat. Nos. 2,929,801; 2,929,802; 2,929,803; 2,929,804; 2,953,839; 2,957,852; 2,962,470; 2,999,839; and 3,009,901.

In some processes for making spandex elastomeric filaments, coalescing jets are used to consolidate the spandex filaments immediately after extrusion. It is also well known that dry-spun spandex filaments are tacky immediately after extrusion. The combination of bringing a group of such tacky filaments together and using a coalescing jet will produce a coalesced multifilament yarn, which is then typically coated with a silicone or other finish before winding to prevent sticking on the package. Such a coalesced grouping of filaments, which is actually a number of tiny individual filaments adhering to one another along their length, is superior in many respects to a single filament of spandex of the same linear density.

The elastomeric filament in the elastomeric single yarn is preferably a continuous filament and can be present in the second yarn in the form of one or more individual filaments or one or more coalesced grouping of filaments. However, it is preferred to use only one coalesced grouping of filaments in the preferred elastomeric single yarn. Whether present as one or more individual filaments or one or more coalesced groupings of filaments, the overall linear density of the elastomer filament(s) in the relaxed state is generally between 17 and 560 dtex (15 and 500 denier) with the preferred linear density range being 44 to 220 dtex (40 to 200 denier).

It is preferred to incorporate the at least one continuous elastomeric filament in the second yarn under tension by drawing or stretching the at least one continuous elastomeric filament prior to the combination with staple fibers by using a slower delivery speed of the at least one continuous elastomeric filament relative to the final second yarn speed. This drawing can be described as the stretch ratio of the continuous elastomeric filament, which is the final second yarn speed divided by the delivery speed of the continuous elastomeric filament.

Typical stretch ratios are 1.5 to 5.0 with 1.5 to 3.50 being preferred. Low stretch ratios yield less elastic recovery while very high stretch ratios make the single yarns difficult to process and the fabric too tight and uncomfortable. The optimum stretch ratio is also dependent on the % weight content of elastomeric core. Tension devices can also be employed to tension and stretch the elastomeric fiber but are less preferred due to the difficulty in reproducing and controlling tension and stretch. The optimum stretch ratio is ultimately determined for each fabric, based on the desired fit and feel of the fabric.

The incorporation of the at least one continuous elastomeric filament into the second yarn of halogenated self-extinguishing staple fibers can be achieved, for example in its simplest practical application, by passing a roving, sliver, or collection of the halogenated self-extinguishing staple fibers through sets of drafting rolls to make a drafted fiber mass to be ring twisted into a single yarn. The at least one continuous elastomeric filament is typically fed from a bobbin through a set of feed rolls and subsequently into the staple fibers prior to the final set of drafting rollers. The slower relative surface speed of the feed rollers to the surface speed of the drafting rollers is increased or decreased to determine the amount of elastic stretch and tension in the final ring-twisted single yarn using conventional techniques.

In some embodiments, the sheath of the at least one second yarn can further comprise heat-resistant polymeric fiber as previously described herein. In some other embodiments, the sheath of the at least one second yarn can further comprise cut-resistant heat-resistant polymeric fiber as previously described herein.

In some embodiments, the sheath of the at least one second yarn can further comprise flame-resistant fiber. By "flame-resistant" fiber, it is meant that a fabric made solely from that fabric has a char length equal to or less than 4 inches and an afterflame equal to or less than 2 seconds per the vertical flame test of ASTM D6143-99. Suitable flame-resistant fibers include aramid fibers, with meta-aramid fibers being especially preferred; the preferred meta-aramid is poly(metaphenylene isophthalamide). Potentially useful flame-resistant fiber include meta-aramid, polyamide-imide, flame-retardant-treated (FR) cellulose, FR cotton, FR lyocell, or mixtures thereof. In some embodiments, the at least one second yarn has preferably 5 weight percent to as much as 35 weight percent flame-resistant fiber, based on the total weight of the polymeric fiber in the at least one second yarn. Also, in some embodiments, the at least one first yarn has preferably 5 weight percent to as much as 35 weight percent flame-resistant fiber, based on the total weight of the polymeric fiber in the at least one first yarn.

Any number of fibers can be included in the second yarn as long the second yarn and the final fabric meets the performance criteria discussed herein.

If used in the second yarn, the heat-resistant polymeric fiber, the cut-resistant heat-resistant polymeric fiber, or the flame-resistant fiber are preferably staple fibers preferably having a length of about 2 to 20 centimeters, preferably about 3.5 to 6 centimeters. Also, if used in the second yarn, the heat-resistant polymeric fiber, the cut-resistant heat-resistant polymeric fiber, and the flame-resistant fiber are preferably staple fibers preferably having a diameter of 5 to 25 micrometers and a linear density of 0.5 to 7 dtex.

In some embodiments, the sheath of the at least one second yarn can further comprise what are known in the art as antistatic fibers or fibers that have the ability to reduce the accumulation of electrical charge in the yarn or in the resultant fabric. In some preferred embodiments the sheath of the at least one second yarn includes at least 1- 5 weight percent antistatic fiber, based on the total weight the at least one second yarn. Preferred antistatic fibers are those that function by the present of carbon in the fiber, either as a carbon coating or carbon particles; especially antistatic fibers that help to eliminate the buildup of charge but are not considered to be electrically conductive in a practical sense. In some embodiments, aramid fiber that contain carbon particles is preferred.

In preferred embodiments the second yarn is free or substantially free of inorganic fibers. The cut-resistant benefits of any inorganic fibers is supplied by the first yarn, eliminating the need for additional inorganic fiber in the second yarn for majority of the intended applications.

In some embodiments, a ply-twisted yarn is formed from the at least first yarn and the at least second yarn. Ply-twisted yarns are made by twisting together at least two individual single yarns. By the phrase "twisting together at least two individual single yarns", it is meant the two single yarns are twisted together without one yarn fully covering the other. This distinguishes ply-twisted yarns from covered or wrapped yarns where a first single yarn is substantially or completely wrapped around a second single yarn so that ideally only the first single yarn is exposed on the surface of the resulting covered yarn.

In one preferred embodiment, the ply-twisted yarn is made from at least two singles yarns, the first singles yarns being (a) the at least one first yarn comprising at least 50 weight percent heat-resistant polymeric fiber, based on the total weight of the first yarn, and wherein at least 30 weight percent of the polymeric fiber present in the at least one first yarn is cut-resistant heat-resistant polymeric fiber having a cut resistance of 500 grams force or higher per ASTM F2992-15, the at least one first yarn further having a sheath/core construction with the sheath comprising the cut-resistant heat-resistant polymeric fiber and the core comprising an inorganic fiber; and the second singles yarn being (b) the at least one second yarn having a sheath/core construction with a sheath of halogenated self-extinguishing staple fibers and a core comprising at least one continuous elastomeric filament, wherein 60 to 95 weight percent of the at least one second yarn is halogenated self-extinguishing fiber, based on the total weight of the second yarn, and the halogenated self-extinguishing fiber is in contact with the at least one continuous elastomeric filament, the second yarn being free or substantially free of inorganic fibers. Each of the single yarns may have some twist.

In some embodiments, the ply-twisted yarns made from the two singles yarns have a total linear density of from 200 to 3000 dtex. The individual staple fibers in either of the singles yarn can have a linear density of 0.5 to 7 dtex, with the preferred linear density range being 1.5 to 3 dtex. The ply-twisted yarns, and the single yarns that make up those ply-twisted yarns, can include other materials as long as the function or performance of the yarn or fabric made from that yarn is not compromised for the desired use.

The ply-twisted yarns can be made from single yarns via the processes disclosed in U.S. Patent No. 6,952,915 to Prickett, and the ply-twisted yarns can have a wide range of ply twist disclosed therein.

The ply-twisted yarns may then be combined with other same or different ply-twisted yarns to form a yarn bundle to form a fabric, or the individual ply-twisted yarns can be used to form the fabric, depending on the desired fabric requirements. For example, two or more of the described ply-twisted yarns can be combined to form a yarn bundle that can be fed to a knitting machine with or without twist. Alternatively, a yarn bundle could be made with one or more of the described ply-twisted yarns with one or more different single yarn to impart desired properties to the final fabric. Since modern knitting machines can knit fabric from a feed of multiple ply-twisted yarns, the bundle of ply-twisted yarns fed to the machine need not have twist, although twist can be put into the bundle if desired.

The at least first yarn used in the preferred ply-twisted yarn when there is no inorganic core is preferably a single 420 dtex (380 denier, equivalent to 14 cotton count) yarn that is ring spun. The yarn has a poly(paraphenylene terephthalamide) (PPD-T) staple sheath, the PPD-T having a 3.8 cm (1.5 inch) cut length and a filament density of 1.7 dtex per filament (1.5 denier per filament).

The at least one second yarn used in the preferred ply-twisted yarn is a single 330 dtex (295 denier, equivalent to 18 cotton count) yarn that is ring-spun. The yarn has a modacrylic staple sheath that at least partially covers the elastomeric core filaments, the modacrylic staple having a 4.8 cm (1.89 inch) cut length and a filament density of 1.7 dtex per filament (1.5 denier per filament). The elastomeric core is a 78 dtex (70 denier) spandex coalesced filament yarn having a 3.0x stretch ratio (approximately 200 percent elongation). In some preferred embodiments, approximately 92 weight percent of the second yarn is comprised of the modacrylic staple and with 8 weight percent of the second yarn being the elastomeric core.

The invention also relates to a cut-resistant woven or knitted fabric made from yarns or a bundle of yarns comprising at least one first yarn and one second yarn. The invention further relates to a cut-resistant woven or knitted fabric made from ply-twisted yarns or a bundle of yarns that includes a ply-twisted yarn, wherein the ply-twisted yarn comprises at least one first yarn and one second yarn as described herein.

Specifically, the invention relates to a cut-resistant woven or knitted fabric made from a ply-twisted yarn made from at least two singles yarns, the first singles yarn being (a) the at least one first yarn comprising at least 50 weight percent heat-resistant polymeric fiber, based on the total weight of the first yarn, and wherein at least 30 weight percent of the polymeric fiber present in the at least one first yarn is cut-resistant heat-resistant polymeric fiber having a cut resistance of 500 grams force or higher per ASTM F2992-15; and the second singles yarn being (b) the at least one second yarn having a sheath/core construction with a sheath of halogenated self-extinguishing staple fibers and a core comprising at least one continuous elastomeric filament, wherein 60 to 95 weight percent of the at least one second yarn is halogenated self-extinguishing fiber, based on the total weight of the second yarn, and the halogenated self-extinguishing fiber is in contact with the at least one continuous elastomeric filament, the second yarn being free or substantially free of inorganic fibers; the fabric having a maximum after-flame time of two seconds or less and weight loss of 5 weight percent of less when tested per NFPA-2112-2018.

In some embodiments, the first singles yarn comprises an at least one first yarn further having a sheath/core construction with the sheath comprising the cut-resistant heat-resistant polymeric fiber and the core comprising an inorganic fiber.

The at least one first yarn and the at least one second yarn work synergistically together in both the yarn and fabric. The at least one continuous elastomeric filament incorporated into the yarn(s) provides improved stretch and recovery, while the heat-resistant staple fibers provide structure in flame and the heat-resistant cut-resistant organic staple fibers and inorganic filaments (if present) provide the yarn and fabric with excellent cut resistance. Fabrics made from such yarn(s) are soft, comfortable and non-abrasive as well as cut resistant.

Ply-twisting of the first yarn with the second yarn is preferred because the ply-twisting helps hold the elastomer single yarn in an extended state without looping upon itself when relaxed. However, if the sheath/core elastomeric single yarn is co-fed with other single yarns in a bundle (without ply-twisting) to a knitting or weaving device with good tension control, an acceptable fabric can be made. When the bundle is comprised of ply-twisted yarns tension control of the yarns while knitting and weaving is less critical.

The preferred fabric is a knit fabric, and any appropriate knit pattern is acceptable. Cut resistance and comfort are affected by tightness of the knit and that tightness can be adjusted to meet any specific need. A very effective combination of cut resistance and comfort for many cut resistant articles has been found in, for example, single jersey and terry knit patterns. The fabrics have a basis weight of about 4 to 30 oz/yd², preferably 6 to 25 oz/yd², the fabrics at the high end of the basis weight range providing more thermal and cut protection.

### Test Methods

Afterflame and Weight Loss were determined according to NFPA 2112-2018 "Standard on Flame-Resistant Clothing for Protection of Industrial Personnel Against Short-Duration Thermal Exposures from Fire", specifically the procedure outline in Section 8.8 of that Standard.

The determination of a "heat resistant polymeric fiber" as discussed herein can be achieved by the use of ASTM E2105-2016 - Standard Practice for General Techniques of Thermogravimetric Analysis (TGA) Coupled With Infrared Analysis (TGA/IR). The analysis of whether or not a synthetic organic polymer retains 90 percent of its original fiber weight is conducted by heating a sample in air to 500° C at a rate of 20° C. per minute.

### Examples

### Knits Made from Ply-Twisted Yarn

Ply-twisted yarns and knits made from the yarns are exemplified in Examples 1, 2, and 3 and Comparative Example A and summarized in Table 6.

### Example 1

A ply-twisted elastic yarn was made by ply twisting a first yarn and a second yarn.

The first yarn was a 14-cotton count sheath-core yarn having a para-aramid fiber sheath and a 50 micron stainless steel wire core, spun on a ring spinning frame. The para-aramid fiber was 2-inch poly(paraphenylene terephthalamide) staple.

The second yarn was an 18-cotton count sheath-core yarn made by core-spinning on a ring-spinning frame of 2-inch modacrylic staple around a 70-denier spandex core; the spandex core was stretched 3X as it was incorporated(spun) into the sheath-core yarn.

The resulting ply-twisted elastic yarn made by ply twisting the first yarn and the second yarn had a total cotton count of 16/2, or 675 denier. Relative amounts of the yarn components are shown in Table 3.

The resulting ply-twisted elastic yarn was knitted into a 13-gauge sleeve on a Shima-Seiki glove knitting machine. The resulting sleeve had excellent hand and form-fitting properties. A fabric sample from resulting sleeve was flame tested in accordance with fire-resistant glove test method detailed in the NFPA-2112-2018 standard. The resulting stretch fabric was found to have 0-seconds of after-flame with 4.8% of the weight consumed during the tests, which was in below the 2-second maximum after-flame requirement and the 5% weight loss limit allowed in the specification.

**Table 3**

| **Component** | **Weight Percent of Ply-twisted yarn (%)** | **Weight Percent in Singles Yarn (%)** |
|---|---|---|
| Para-aramid Fiber | 36.4 | 65 |
| Steel Wire | 19.8 | 35 |
| Modacrylic Fiber | 40.3 | 92 |
| Elastic Fiber | 3.5 | 8 |

### Example 2

The ply-twisted elastic yarn of Example 1 was repeated, with the following exceptions.

The first yarn was a 26-cotton count yarn having a para-aramid fiber sheath and a stainless steel wire core made with a 35 micron stainless steel wire core. The second yarn was a 32-cotton count yarn having a modacrylic sheath and a 40-denier spandex core that was stretched 3X during spinning.

As in Example 1, the resulting ply-twisted elastic yarn made by ply twisting the first yarn and the second yarn had a total cotton count of 29/2, or 371 denier. Relative amounts of the yarn components are shown in Table 4.

The resulting ply-twisted elastic yarn was knitted into an 18-gauge sleeve on a Shima-Seiki glove knitting machine. The resulting sleeve had excellent form-fitting properties. A fabric sample from the resulting sleeve was washed to remove knitting oils and finishes and flame tested in accordance with fire-resistant glove test method detailed in the NFPA-2112-2018 standard. The resulting stretch fabric was found to have 0 seconds of after-flame with 3.3 % of the weight consumed during the tests, which was in below the 2-second maximum after-flame requirement and the 5% weight loss limit allowed in the specification.

**Table 4**

| **Component** | **Weight Percent of Ply-twisted yarn (%)** | **Weight Percent in Singles Yarn (%)** |
|---|---|---|
| Para-aramid Fiber | 37.4 | 68 |
| Steel Wire | 17.8 | 32 |
| Modacrylic Fiber | 41.2 | 92 |
| Elastic Fiber | 3.6 | 8 |

### Example 3

The ply-twisted elastic yarn of Example 1 was repeated, with the following exceptions.

The first yarn was a 19.5-cotton count yarn having a para-aramid fiber sheath and a stainless steel wire core made with a 45 micron stainless steel wire core that was stretched 3X during spinning. The second yarn was a 32-cotton count sheath-core yarn having a 40-denier spandex core; however, the sheath was a blend of 82 weight % modacrylic staple fiber and 10 weight percent of a 2-inch cut-length meta-aramid staple fiber blend; specifically, the meta-aramid blend contained 93 weight % poly(metaphenylene isophthalamide) staple fiber, 5 weight % poly(paraphenylene terephthalamide) staple, and 2 weight % carbon-core nylon antistatic fiber.

As in Example 1, the resulting ply-twisted elastic yarn made by ply twisting the first yarn and the second yarn had a total cotton count of 24/2, or 439 denier. Relative amounts of the yarn components are shown in Table 5.

The resulting ply-twisted elastic yarn was knitted into an 18-gauge sleeve on a Shima-Seiki glove knitting machine. The resulting sleeve had excellent form-fitting properties.

A fabric sample of the sleeve that was produced was washed to remove knitting oils and finishes and then flame tested in accordance with fire-resistant glove test method detailed in the NFPA-2112-2018 standard. The resulting stretch fabric was found to have 0-seconds of after-flame with 3.9% of the weight consumed during the tests, which was in below the 2-second maximum after-flame requirement and the 5% weight loss limit allowed in the specification.

Another fabric sample of the sleeve that was produced was flame tested in accordance with fire-resistant glove test method detailed in the EN407:2020 standard. The resulting stretch fabric was found to have 0-seconds of after-flame and 0-seconds of after-glow after 3 seconds and 15 seconds of exposure to the flame, which was in below the 2-second maximum after-flame and 5-second maximum after-glow requirement to achieve the highest ranking described in the specification.

**Table 5**

| **Component** | **Weight Percent of Ply-twisted yarn (%)** | **Weight Percent in Singles Yarn (%)** |
|---|---|---|
| Para-Aramid Fiber | 37.3 | 60 |
| Steel Wire | 24.9 | 40 |
| Modacrylic Fiber | 31.0 | 82 |
| Meta-Aramid Fiber* | 3.8 | 10 |
| Elastic Fiber | 3.0 | 8 |

| | | |
|---|---|---|
| *Actual blend of 93 wt% meta-aramid fiber, 5 wt% para-aramid fiber, and 2 wt% carbon-core nylon antistatic fiber. | | |

### Comparative Example A

A comparative ply-twisted elastic yarn similar to that of Example 3 was made; however, the first yarn having a para-aramid fiber sheath and a stainless steel wire core was made with 1.5-inch poly(paraphenylene terephthalamide) staple and a 45-micron stainless steel wire core. The second yarn, which was again a 32-cotton count sheath-core yarn, had a sheath of solely 1.5 inch cut-length nylon staple core-spun around the 40-denier spandex core.

The resulting 24's-2 count ply-twisted yarn was knitted into an 18-gauge sleeve on a Shima-Seiki glove knitting machine. The resulting sleeve had excellent form fitting properties.

However, the sample produced was flame tested in accordance with fire-resistant glove test method detailed in the EN407:2020 standard. The resulting stretch fabric was found to have at least 25-seconds of after-flame after 3 seconds of exposure to the flame, which was higher than 20-second maximum after-flame requirement to achieve even the lowest ranking described in the specification.

Because of the excessive afterflame with only 3-seconds of flame exposure, subsequent testing was not done for 15-second exposure in the EN407 test nor the 12-second exposure in the NFPA-2112 test.

**Table 6**

| **Ex.** | **Yarn Type** | **Knit Type** | **First Yarn** | **Second Yarn** | **After Flame (sec)** | **Weight Loss %** |
|---|---|---|---|---|---|---|
| **1** | One Ply-Twisted Yarn | 13 Gauge Knit | Para-Aramid Sheath/ Steel Core | Modacrylic Sheath/ Spandex Core | 2 | 4.8 |
| **2** | One Ply-Twisted Yarn | 18 Gauge Knit | Para-Aramid Sheath/ Steel Core | Modacrylic Sheath/ Spandex Core | 0 | 3.3 |
| **3** | One Ply-Twisted Yarn | 18 Gauge Knit | Para-Aramid Sheath/ Steel Core | Modacrylic +Meta-Aramid Sheath/ Spandex Core | 0 | 3.9 |
| **A** | One Ply-Twisted Yarn | 18 Gauge Knit | Para-Aramid Sheath/ Steel Core | Nylon Sheath/ Spandex Core | >25 | NA |

### Knits Made by Co-Knitting Two Parallel Ends

Knits made from co-knitting the yarns by supplying individual ends or a bundle of individual end to knitting machine are exemplified in Example 4 and Comparative Examples B and summarized in Table 4.

### Example 4

A first end that is a 2-ply para-aramid ring spun yarn, each ply yarn made from 2-inch poly(paraphenylene terephthalamide) staple yarns, with each of the 2 ply yarns having a 16 cotton count; was co-knitted with a second end that was the 18 cotton count sheath-core yarn of Example 1.

The two ends were then co-knit two-ends in into a sleeve on a 13-gauge knitting machine. The resulting sleeve had excellent hand and form fitting properties.

A fabric sample of the produced sleeve was washed to remove knitting oils and finishes and flame tested in accordance with fire-resistant glove test method detailed in the NFPA-2112-2018 standard. The resulting stretch fabric was found to have 0-seconds of after-flame with 2.5% of the weight consumed during the tests, which was in below the 2-second maximum after-flame requirement and the 5% weight loss limit allowed in the specification.

### Comparative Example B

An end of 12 cotton count modacrylic ring spun yarn, made from 2-inch modacrylic staple, was co-knitted with an end of 18 cotton count sheath-core yarn of Example 1. The two ends were co-knitted two-ends in into a sleeve on a 13-gauge knitting machine. The resulting sleeve had excellent hand and form fitting properties.

The sample produced was washed to remove knitting oils and finishes and flame tested in accordance with fire-resistant glove test method detailed in the NFPA-2112-2018 standard. The resulting stretch fabric was found to have 2.3-seconds of after-flame with 5.8% of the weight consumed during the tests, which was above the 2-second maximum after-flame requirement and the 5% weight loss limit allowed in the specification.

**Table 7**

| **Ex.** | **Yarn Type** | **Knit Type** | **First Yarn** | **Second Yarn** | **After Flame (sec)** | **Weight Loss %** |
|---|---|---|---|---|---|---|
| **4** | One Ply-Twisted Yarn | 13 Gauge Knit | Para-Aramid Singles Yarn Plied with Para-Aramid Singles Yarn | Modacrylic Sheath/ Spandex Core | 0 | 4.8 |
| **B** | One Ply-Twisted Yarn | 13 Gauge Knit | Modacrylic Singles Yarn | Modacrylic Sheath/ Spandex Core | 2.3 | 5.8 |

### Knits Made from Weft-Insertion

Knits made from co-knitting the yarns via weft-insertion are exemplified in Example 3 and Comparative Examples B & C and summarized in Table 4.

### Example 5

A first end, that is a 2-ply para-aramid ring spun yarn, each ply yarn made from 2-inch poly(paraphenylene terephthalamide) staple yarns, with each of the two ply yarns having a 16 yarn count, was co-knitted with a second end that was a modacrylic sheath-spandex core elastic yarn, made by ring-spinning a 1200 denier core-spun fiber, with a 440 denier spandex core, that was stretched 3X during the yarn spinning process, to produce a fire-resistant yarn. The composition of the elastic core yarn was approximately 12% spandex and 88% modacrylic staple fiber.

The first and second ends were co-knitted into a 13-gauge knitted sleeve cuff on a Shima-Seiki flatbed knitted machine, using a weft insertion technique that inserted in every third stitch the modacrylic sheath-spandex core elastic yarn. The resulting sleeve had excellent form fitting properties.

The sample produced was washed to remove knitting oils and finishes and flame tested in accordance with fire-resistant glove test method detailed in the NFPA-2112-2018 standard. The resulting stretch fabric was found to have 0-seconds of after-flame with 4% of the weight consumed during the tests, which was in below the 2-second maximum after-flame requirement and the 5% weight loss limit allowed in the specification.

### Comparative Example C

The 2-ply para-aramid ring spun yarn first end of Example 5 was combined was a different second end, that second end being a polyester fiber wrapped-covered rubber elastic cord from Supreme Elastic Corporation, and the first and second ends were co-knitted to produce an elastic cuff on a Shima-Seiki flatbed knitted machine. The elastic cord composition was estimated to be 75% polyester fiber and 25% rubber. The ends were co-knitted using a weft insertion technique that inserted the polyester fiber wrapped-covered rubber elastic cord in every third stitch of the 13-gauge knitted sleeve. The resulting sleeve had excellent form-fitting properties.

A fabric sample from the produced sleeve was washed to remove knitting oils and finishes and flame tested in accordance with fire-resistant glove test method detailed in the NFPA-2112-2018 standard. The resulting fabric was found to have 43-seconds of after-flame with 9% of the weight consumed during the tests, which was in excess of the 2-second maximum after-flame and 5% weight loss limit allowed in the specification.

### Comparative Example D

4-ends of a ring spun yarn, made from 2-inch modacrylic staple, with each yarn having a 35 cotton count, was co-knitted with a sheath-core elastic yarn having a modacrylic sheath and spandex core. The sheath-core elastic yarn was made by ring-spinning a 1200 denier modacrylic staple yarn with a 440 denier spandex core, while the spandex was stretched 3X during spinning to produce the sheath-core elastic yarn having a composition that was approximately 12% spandex and 88% modacrylic staple fiber. The elastic yarn was co-knitted using a weft insertion technique in every third stitch of the 13-gauge knitted sleeve being knitted on the glove knitting machine. The resulting sleeve had excellent form fitting properties.

A fabric sample from the produced sleeve was washed to remove knitting oils and finishes and flame tested in accordance with fire-resistant glove test method detailed in the NFPA-2112-2018 standard. The resulting stretch fabric was found to have 0-seconds of after-flame with 10% of the weight consumed during the tests, which was in below the 2-second maximum after-flame requirement but above the 5% weight loss limit allowed in the specification.

**Table 8**

| **Ex.** | **Yarn Type** | **Knit Type** | **First Yarn** | **Second Yarn** | **After Flame (sec)** | **Weight Loss %** |
|---|---|---|---|---|---|---|
| **5** | Two Ends | 13 Gauge Co-Knit using weft insertion | Ply-Twisted Para-Aramid/ Para-Aram id | Modacrylic Sheath/ Spandex Core | 0 | 4 |
| **C** | Two Ends | 13 Gauge Co-Knit using weft insertion | Ply-Twisted Para-Aramid/ Para-Aram id | Polyester Sheath/ Rubber Core | 43 | 9 |
| **D** | Four Ends | 13 Gauge Co-Knit using weft insertion | Separate Modacrylic Yarns | Modacrylic Sheath/ Spandex Core | 0 | 10 |

## Claims

1. A flame-resistant cut-resistant fabric, comprising:
(a) at least one first yarn comprising at least 50 weight percent heat-resistant polymeric fiber, based on the total weight of the polymeric fiber in the first yarn, wherein at least 30 weight percent of the polymeric fiber present in the at least one first yarn is cut-resistant heat-resistant polymeric fiber having a cut resistance of 4.9 N (500 grams force) or higher per ASTM F2992-15; and
(b) at least one second yarn having a sheath/core construction with a core comprising at least one continuous elastomeric filament, the second yarn being free of inorganic fibers,
the fabric being **characterized in that** the sheath of the second yarn comprises halogenated self-extinguishing stable fibers, 60 to 95 weight percent of the at least one second yarn is halogenated self-extinguishing fiber, based on the total weight of the second yarn, and the halogenated self-extinguishing fiber is in contact with the at least one continuous elastomeric filament, and **in that** the fabric has a maximum after-flame time of two seconds or less and weight loss of 5 weight percent of less when tested per NFPA-2112-2018.

2. The fabric of claim 1, wherein the at least one first yarn has a sheath/core construction with a sheath comprising the cut-resistant heat-resistant polymeric fiber and a core comprising an inorganic fiber, wherein the inorganic fiber is preferably metal filament or is preferably glass filament.

3. The fabric of claim 1 or 2, wherein the heat-resistant polymeric fiber or the cut-resistant heat-resistant polymeric fiber is aramid copolymer, para-aramid, polybenzazole, polybenzimidazole, polyimide or mixtures thereof, preferably wherein the heat-resistant polymeric fiber or the cut-resistant heat-resistant polymeric fiber is para-aramid, which preferably is poly(paraphenylene terephthalamide.

4. The fabric of any one of claims 1 to 3, wherein the at least one first yarn further comprises a flame resistant fiber that is not cut-resistant, wherein preferably the flame resistant fiber is meta-aramid, polyamide-imide, flame-retardant-treated (FR) cellulose, FR cotton, FR lyocell, or mixtures thereof, more preferably meta-aramid, which even more preferably is poly(metaphenylene isophthalamide).

5. The fabric of any one of claims 1 to 4, wherein 80 to 95 weight percent of the total weight of the at least one second yarn is the halogenated self-extinguishing fiber.

6. The fabric of any one of claims 1 to 5, wherein the halogenated self-extinguishing fiber is modacrylic fiber.

7. The fabric of any one of claims 1 to 6, wherein 5 to 40 weight percent of the total weight of the at least one second yarn is the at least one continuous elastomeric filament.

8. The fabric of any one of claims 1 to 7, wherein the at least one continuous elastomeric filament is spandex filament.

9. The fabric of any one of claims 1 to 8 wherein the sheath of the at least one second yarn further comprises heat-resistant polymeric fiber.

10. The fabric of any one of claims 1 to 9, wherein the sheath of the at least one second yarn further comprises a flame resistant fiber that is not cut-resistant, wherein preferably the flame resistant fiber is meta-aramid, polyamide-imide, flame-retardant-treated (FR) cellulose, FR cotton, FR lyocell, or mixtures thereof, more preferably meta-aramid, which preferably is poly(metaphenylene isophthalamide).

11. The fabric of any one of claims 1 to 10, wherein the sheath of the at least one second yarn further comprises an antistatic fiber.

12. The fabric of any one of claims 1 to 11 comprising a ply-twisted yarn of the at least one first yarn and the at least one second yarn.

13. The fabric of any one of claims 1-12 wherein the fabric is a knit fabric.

14. The fabric of any one of claims 1-11 having co-knit structure of the at least one first yarn and the at least one second yarn, wherein preferably the at least one first yarn and the at least one second yarn are in a parallel relationship to one another in the co-knit structure, or wherein preferably the at least one second yarn is a weft insertion in the co-knit structure.

15. A glove or other article comprising the fabric of any one of claims 1-14.

## Patentansprüche

1. Flammbeständiger, schnittfester Textilstoff, umfassend:
(a) mindestens ein erstes Garn, das mindestens 50 Gewichtsprozent hitzefeste polymere Faser, auf das Gesamtgewicht der polymeren Faser in dem ersten Garn bezogen, umfasst, wobei mindestens 30 Gewichtsprozent der polymeren Faser, die in dem mindestens einen ersten Garn vorliegt, schnittfeste hitzefeste polymere Faser ist, die eine Schnittfestigkeit von 4,9 N (500 Pond) oder höher ASTM F2992-15 entsprechend aufweist; und
(b) mindestens ein zweites Garn, das eine Mantel-/Kern-Konstruktion mit einem Kern aufweist, der mindestens ein kontinuierliches elastomeres Filament umfasst,
wobei das zweite Garn frei von anorganischen Fasern ist,
wobei der Textilstoff **dadurch gekennzeichnet ist, dass** der Mantel des zweiten Garns halogenierte selbstlöschende Stapelfasern umfasst,
60 bis 95 Gewichtsprozent des mindestens einen zweiten Garns halogenierte selbstlöschende Stapelfaser, auf das Gesamtgewicht des zweiten Garns bezogen, ist und die halogenierte selbstlöschende Faser in Kontakt mit dem mindestens einen kontinuierlichen elastomeren Filament steht, und dadurch, dass
der Textilstoff eine maximale Nachflammzeit von zwei Sekunden oder weniger und einen Gewichtsverlust von 5 Gewichtsprozent oder weniger, wenn NFPA-2112-2018 entsprechend getestet, aufweist.

2. Textilstoff nach Anspruch 1, wobei das mindestens eine erste Garn eine Mantel-/Kernkonstruktion aufweist, wobei ein Mantel die schnittfeste hitzefeste polymere Faser umfasst und ein Kern eine anorganische Faser umfasst, wobei die anorganische Faser bevorzugt Metallfilament ist oder bevorzugt Glasfilament ist.

3. Textilstoff nach Anspruch 1 oder 2, wobei die hitzefeste polymere Faser oder die schnittfeste hitzefeste polymere Faser Aramidcopolymer, Para-Aramid, Polybenzazol, Polybenzimidazol, Polyimid oder Mischungen davon ist, wobei bevorzugt die hitzefeste polymere Faser oder die schnittfeste hitzefeste polymere Faser Para-Aramid ist, das bevorzugt Poly(paraphenylenterephthalamid) ist.

4. Textilstoff nach einem der Ansprüche 1 bis 3, wobei das mindestens eine erste Garn ferner eine flammbeständige Faser umfasst, die nicht schnittfest ist, wobei die flammbeständige Faser bevorzugt Meta-Aramid, Polyamidimid, flammhemmend behandelte (FH) Cellulose, FH-Baumwolle, FH-Lyocell oder Mischungen davon, noch bevorzugter Meta-Aramid ist, das selbst noch bevorzugter Poly(metaphenylenisophthalamid) ist.

5. Textilstoff nach einem der Ansprüche 1 bis 4, wobei 80 bis 95 Gewichtsprozent des Gesamtgewichts des mindestens einen zweiten Garns die halogenierte selbstlöschende Faser ist.

6. Textilstoff nach einem der Ansprüche 1 bis 5, wobei die halogenierte selbstlöschende Faser Modacrylfaser ist.

7. Textilstoff nach einem der Ansprüche 1 bis 6, wobei 5 bis 40 Gewichtsprozent des Gesamtgewichts des mindestens einen zweiten Garns das mindestens eine kontinuierliche elastomere Filament ist.

8. Textilstoff nach einem der Ansprüche 1 bis 7, wobei das mindestens eine kontinuierliche elastomere Filament Spandexfilament ist.

9. Textilstoff nach einem der Ansprüche 1 bis 8, wobei der Mantel des mindestens einen zweiten Garns ferner hitzefeste polymere Faser umfasst.

10. Textilstoff nach einem der Ansprüche 1 bis 9, wobei der Mantel des mindestens einen zweiten Garns ferner eine flammbeständige Faser umfasst, die nicht schnittfest ist, wobei bevorzugt die flammbeständige Faser Meta-Aramid, Polyamidimid, flammhemmend behandelte (FH) Cellulose, FH-Baumwolle, FH-Lyocell oder Mischungen davon, noch bevorzugter Meta-Aramid ist, das bevorzugt Poly(metaphenylenisophthalamid) ist.

11. Textilstoff nach einem der Ansprüche 1 bis 10, wobei der Mantel des mindestens einen zweiten Garns ferner eine antistatische Faser umfasst.

12. Textilstoff nach einem der Ansprüche 1 bis 11, umfassend ein doppelt gezwirntes Garn des mindestens einen ersten Garns und des mindestens einen zweiten Garns.

13. Textilstoff nach einem der Ansprüche 1 bis 12, wobei der Textilstoff ein gestrickter Textilstoff ist.

14. Textilstoff nach einem der Ansprüche 1 bis 11, der eine zusammengestrickte Struktur aus dem mindestens einen ersten Garn und dem mindestens einen zweiten Garn aufweist, wobei bevorzugt das mindestens eine erste Garn und das mindestens eine zweite Garn sich in einem parallelen Verhältnis zueinander in der zusammengestrickten Struktur befinden oder wobei bevorzugt das mindestens eine zweite Garn ein Schusseinschub in die zusammengestrickte Struktur ist.

15. Handschuh oder anderer Artikel, der den Textilstoff nach einem der Ansprüche 1 bis 14 umfasst.

## Revendications

1. Tissu résistant à la coupure et au feu comprenant :
(a) au moins un premier fil comprenant au moins 50 pour cent en poids de fibre polymère résistante à la chaleur, sur la base du poids total de la fibre polymère dans le premier fil, dans lequel au moins 30 pour cent en poids de la fibre polymère présente dans l'au moins un premier fil est une fibre polymère résistante à la chaleur et résistante aux coupures présentant une résistance aux coupures de 4,9 N (500 grammes-force) ou plus selon la norme ASTM F2992-15 ; et
(b) au moins un deuxième fil présentant une structure gaine/noyau avec un noyau comprenant au moins un filament élastomère continu,
le deuxième fil étant dénué de fibres inorganiques,
le tissu étant **caractérisé en ce que** la gaine du second fil comprend une fibre discontinue autoextinguible halogénée,
60 à 95 pour cent en poids de l'au moins un deuxième fil est constitué d'une fibre discontinue autoextinguible halogénée, sur la base du poids total du deuxième fil, et la fibre autoextinguible halogénée est en contact avec l'au moins un filament élastomère continu, et **en ce que**
le tissu présente une persistance de flamme maximale de deux secondes ou moins et une perte de poids de 5 pour cent en poids ou moins lors d'un test selon la norme NFPA-2112-2018.

2. Tissu selon la revendication 1, dans lequel l'au moins un premier fil présente une structure gaine/noyau avec une gaine comprenant la fibre polymère résistante à la chaleur et résistante aux coupures et un noyau comprenant une fibre inorganique, dans lequel la fibre inorganique est de préférence un filament métallique ou est de préférence un filament en verre.

3. Tissu selon la revendication 1 ou la revendication 2, dans lequel la fibre polymère résistante à la chaleur ou la fibre polymère résistante à la chaleur et résistante aux coupures est un copolymère d'aramide, un para-aramide, un polybenzazole, un polybenzimidazole, un polyimide ou des mélanges correspondants, de préférence dans lequel la fibre polymère résistante à la chaleur ou la fibre polymère résistante à la chaleur et résistante à la coupure est un para-aramide, qui est de préférence un poly(paraphénylène téréphtalamide).

4. Tissu selon l'une quelconque des revendications 1 à 3, dans lequel l'au moins un premier fil comprend en outre une fibre résistante au feu qui n'est pas résistante aux coupures, de préférence dans lequel la fibre résistante au feu est un méta-aramide, un polyamide-imide, une cellulose traitée ignifuge (IF), un coton IF, un lyocell IF, ou des mélanges correspondants, plus préférablement un méta-aramide, qui, de manière encore davantage préférée, est un poly(métaphénylène isophtalamide).

5. Tissu selon l'une quelconque des revendications 1 à 4, dans lequel 80 à 95 pour cent en poids du poids total de l'au moins un second fil est la fibre autoextinguible halogénée.

6. Tissu selon l'une quelconque des revendications 1 à 5, dans lequel la fibre autoextinguible halogénée est une fibre de modacrylique.

7. Tissu selon l'une quelconque des revendications 1 à 6, dans lequel 5 à 40 pour cent en poids du poids total de l'au moins un second fil est l'au moins un filament élastomère continu.

8. Tissu selon l'une quelconque des revendications 1 à 7, dans lequel l'au moins un filament élastomère continu est un filament de spandex.

9. Tissu selon l'une quelconque des revendications 1 à 8, dans lequel la gaine de l'au moins un deuxième fil comprend en outre une fibre polymère résistante à la chaleur.

10. Tissu selon l'une quelconque des revendications 1 à 9, dans lequel la gaine de l'au moins un deuxième second fil comprend en outre une fibre résistante au feu qui n'est pas résistante à la coupure, dans lequel de préférence la fibre résistante au feu est un méta-aramide, un polyamide-imide, une cellulose traitée ignifuge (IF), un coton IF, un lyocell IF, ou des mélanges de ceux-ci, plus préférablement un méta-aramide, qui est de préférence un poly(métaphénylène isophtalamide).

11. Tissu selon l'une quelconque des revendications 1 à 10, dans lequel la gaine de l'au moins un deuxième fil comprend en outre une fibre antistatique.

12. Tissu selon l'une quelconque des revendications 1 à 11, comprenant un fil à torsion retors de l'au moins un premier fil et le au moins un second fil.

13. Tissu selon l'une quelconque des revendications 1 à 12, dans lequel le tissu est un tissu tricoté.

14. Tissu selon l'une quelconque des revendications 1 à 11, présentant une structure co-tricotée de l'au moins un premier fil et l'au moins un deuxième fil, dans lequel, de préférence, l'au moins un premier fil et l'au moins un deuxième fil sont dans une relation en parallèle l'un par rapport à l'autre dans la structure co-tricotée, ou dans lequel, de préférence l'au moins un deuxième fil est une insertion de trame dans la structure co-tricotée.

15. Gant ou autre article comprenant le tissu selon l'une quelconque des revendications 1 à 14.
